

## [54] HIGH PERFORMANCE BLOCKING ELECTRODE FOR ELECTROPHOTOPHORESIS

3,744,896 7/1973 Carreira ..... 355/3 P  
3,776,628 12/1973 Gundlach ..... 355/3 P

[75] Inventors: Addison C. Scheckler, Cato; Luke C. Lin, Rochester, both of N.Y.

Primary Examiner—J. D. Miller  
Assistant Examiner—Harry E. Moose, Jr.

[73] Assignee: Xerox Corporation, Stamford, Conn.

[22] Filed: Feb. 15, 1973

[21] Appl. No.: 332,974

[52] U.S. Cl. .... 317/262 A, 204/300, 355/3 P

[51] Int. Cl. .... H01t 19/00

[58] Field of Search..... 204/280, 299, 300;  
355/3 P; 317/262 A; 96/1.2, 1.3

## [56] References Cited

## UNITED STATES PATENTS

3,551,320 12/1970 Krieger et al. .... 317/262

## [57] ABSTRACT

Compositions suited for use as a blocking electrode material in a photoelectrophoretic imaging process are disclosed. These compositions comprise a mixture of a polymeric material and a finely divided ferroelectric filler such as a metal titanate or stannate. Blocking electrodes so prepared exhibit the high dielectric constant and high dielectric strength which are desirable in a blocking electrode.

15 Claims, 4 Drawing Figures



PATENTED JAN 7 1975

3,859,576



FIG. 1



FIG. 2



FIG. 3



FIG. 4

# HIGH PERFORMANCE BLOCKING ELECTRODE FOR ELECTROPHOTOPHORESIS

## BACKGROUND OF THE INVENTION

The invention relates to imaging systems and, in particular, to photoelectrophoretic imaging systems employing novel blocking electrodes.

In the photoelectrophoretic imaging process, an image is formed from an imaging suspension or ink by subjecting the ink to an electric field and exposing it to activating electromagnetic radiation, e.g., light in the visible spectrum. The imaging suspension is composed of light sensitive particles suspended within an insulating liquid carrier. The particles are believed to bear a net electrical charge while in suspension and during imaging. Conventionally, the ink is placed between electrodes used to establish the electric field and is exposed to a light image through one of the electrodes which is at least partially transparent. According to one theory, particles attracted to the transparent injecting electrode by the electric field exchange charge, directly or indirectly, with the injecting electrode when exposed to light, and migrate under the influence of the field through the liquid carrier toward the opposite electrode. As a result of the migration, positive and negative images are formed on the two electrodes.

The photoelectrophoretic imaging process is either monochromatic or polychromatic, depending upon whether the light sensitive particles within the liquid carrier are responsive to the same or different portions of the light spectrum. A full color polychromatic system is obtained, for example, by using cyan, magenta and yellow colored particles which are responsive to red, green and blue light, respectively. An extensive and detailed description of the photoelectrophoretic process is found in U.S. Pat. Nos. 3,384,565 and 3,384,484 to Tulagin and Carreira; 3,383,993 to Yeh and 3,384,566 to Clark, all of which are incorporated herein by reference.

A high field between the electrodes is required for efficient imaging. However, a high field increases the possibility of dielectric breakdown of the imaging suspension, possible damage to the injecting electrode, and loss of image quality. One method of overcoming this problem is to interpose a layer of high resistivity material, i.e., greater than about 10<sup>7</sup> ohm-cm, between the imaging suspension on the injecting electrode and the opposite electrode. This layer of high resistivity material in association with the conductive support which forms the electrode opposite the injecting electrode is known as the blocking electrode. The blocking electrode functions as a current limiting device and prevents significant charge exchange between it and the particles of the ink suspension which have migrated to its surface during the imaging process.

Besides being of the requisite resistivity, the blocking layer must also be able to withstand a high electric flux density generated during the imaging process. For best results in terms of image quality, a high electric field ordinarily in the order of greater than 10<sup>7</sup> volts per meter is generated in the ink. Thus, during imaging if the blocking layer and ink system were to be regarded as two resistance/capacitance circuits in series, it is important that the dielectric breakdown strength and dielectric constant of the blocking layer be sufficiently high to support the high field generated.

Where the blocking electrode is subject to cyclic reuse as, for example, in the embodiment shown in FIG. 1, the resistivity of the blocking layer should not be so high that residual charges present on the surface of the layer after one cycle are unable to dissipate via internal conduction prior to undergoing a second and subsequent cycle.

These factors, plus other factors such as durability, mechanical strength, solvent resistance, and compliance are often at odds with one another. For example, some materials such as elastomers and plastics may possess requisite high dielectric strength and mechanical properties, but have a low dielectric constant, generally in the order of less than eight or a resistivity in excess of that desired in a blocking material used in a cycle process. On the other hand, a material such as Baryta paper, which consists of paper coated with barium sulfate suspended in a gelatin solution, leaves something to be desired in terms of mechanical strength, compliance and durability.

Accordingly, it is a primary object of this invention to define a blocking electrode incorporating the above and other advantageous chemical, mechanical and electrical properties.

Yet another object of the invention is the enhancement of the photoelectrophoretic process.

A specific object of this invention is to build a blocking electrode having a polymeric blocking layer having good compliance, high dielectric strength, high dielectric constant and relatively short time constant.

Another object of the present invention is to develop embodiments of the photoelectrophoretic process that tend to optimize the parameters and/or overcome the limitations of the blocking electrode.

## SUMMARY OF THE INVENTION

The foregoing and other objects of the invention are realized by preparing blocking electrode material comprising a polymeric matrix material having incorporated therein effective amounts of a finely divided ferroelectric material or a mixture of ferroelectric materials sufficient to enhance the electrical properties of the polymeric material for use in an electrophoretic imaging process. Preferred ferroelectrics are those materials having a dielectric constant of from about 15 to 10,000 (10<sup>6</sup> Hertz) or more, such as alkaline earth metal titanates or stannates. More preferred are ferroelectrics having a dielectric constant in excess of about 100, such as barium or strontium titanate. The blocking electrode encompassing the blocking layer of the present invention may be in the form of a conductive roller connected to a source of potential and having a film of the blocking layer adhered to its surface, as in FIGS. 1 and 2. The blocking electrode may also be in the form of an endless belt comprising a conductive material connected to a source of potential underlying a layer of the blocking material, as in FIG. 3. The blocking electrode may also take the form of a web comprising a roll-fed sheet of the blocking material which is superimposed between an injecting electrode and a conductive backing electrode, an embodiment of which is shown in FIG. 4.

Where the polymeric blocking material containing the ferroelectric exhibits a volume resistivity in excess of about 10<sup>13</sup> ohm-cm and is intended for use in a continuous process involving continuous cyclic exposure of the same surface to the imaging process as in FIG.

1 for example, it has been found that the electrical properties of the blocking material may be further enhanced by additionally including minor amounts of a material more conductive than the polymeric material used in fabricating the blocking layer. Examples of suitable materials are graphite, conductive carbon black, Lewis acids, plasticizers, polyelectrolytic resins and the like.

2 The polymeric blocking layer may be applied to the appropriate conductive substrate by any method such as dip or roller coating, by laminating a sheet or film of the material to the conductive substrate or by heat shrinking where the substrate is a roller or drum and the polymeric material is susceptible to heat shrinkage. Alternatively, the polymeric blocking layer may be fabricated into a web or sheet adapted to be fed into intimate contact with a conductive substrate.

#### DETAILED DESCRIPTION OF THE DRAWINGS

3 Other objects and features of the present invention will become apparent upon the reading of the present disclosure and from the drawings which illustrate several of the environments in which the polymeric blocking layers of this invention are used.

4 FIGS. 1 and 2 are schematic side sectional views of a photoelectrophoretic imaging system wherein the blocking electrode is in a roller configuration.

5 FIG. 3 is a schematic side sectional view wherein the blocking electrode is in the form of an endless web or belt.

6 FIG. 4 is a schematic side sectional view of an embodiment wherein the blocking electrode is formed by passing a web of blocking material over a conductive electrode.

#### DETAILED DESCRIPTION OF THE INVENTION

7 In order to more thoroughly understand the role of the blocking electrode material of this invention in photoelectrophoretic imaging processes, a discussion of several exemplary systems is warranted.

8 Referring now to FIG. 1, there is seen a transparent electrode generally designated as 11 which in this case is made up of a layer of optically transparent glass 12 overcoated with a thin optically transparent layer 13 of tin oxide. This oxide coated glass is commercially available under the trade name NESA glass from Pittsburgh Plate Glass Company, Pittsburgh, Pa. This base electrode is referred to as the injecting electrode. Coated on the layer of electrode 11 is a thin layer of finely divided photosensitive particles dispersed in an insulating carrier liquid. This suspension 14 may also contain sensitizers and/or binders for the particles which are dissolved or suspended in the carrier liquid along with the particles. Adjacent electrode 11 is a roller electrode 23 which is connected to one side of a potential source 17 through a switch 18 with the opposite side of the potential source being connected to the tin oxide coating on electrode 11 so that when switch 18 is closed an electric field is applied across the liquid suspension as electrode 23 rolls across the surface of electrode 11 in the direction indicated by the arrow in the drawing. Electrode 23 is made up of a central core 24 which is preferably of fairly high electrical conductivity and is covered with a layer of blocking electrode material 26. An image projector made up of light source 19, a transparency 21 and a lens 22 is provided to exposed suspension 14 to a light image of the original transparency 21

9 to be reproduced. In imaging the roller 23 is caused to roll across the top surface of electrode 11 with switch 18 closed during the period of exposure. This exposure causes exposed particles originally on electrode 11 to migrate through the liquid and adhere to the surface of the blocking electrode leaving behind a particle image on the injecting electrode surface which is a duplicate of the original transparency 19. This image may then be fixed in place as, for example, by placing a lamination over its top surface or by virtue of a dissolved binder material in the carrier liquid such as a paraffin wax or other suitable binder that comes out of solution as the carrier liquid evaporates. In fact, the carrier liquid itself may be a molten paraffin wax or other suitable binder in a liquid state which is self-fixing upon cooling and return to the solid state. In the alternative, the particle image remaining on the electrode 11 may be transferred to another surface and fixed thereon, if desired. The system has been found to be capable of producing either monochromatic or polychromatic images depending upon the color, sensitivity and number of different pigments suspended in the carrier liquid and the color light to which the suspension is exposed.

10 In FIG. 2 there is shown an apparatus whereby a large broad area "tracking" contact is made by the blocking electrode with the imaging suspension 14 during the imaging process. Like numerals have been used to identify like elements throughout FIGS. 2 to 4 where they correspond with the elements of the FIG. 1 device, 15 and as can be seen from FIG. 2, this device is identical with that of FIG. 1 with the exception of the blocking electrode structure wherein a roller, generally designated 29, is employed. This roller electrode 29 consists of a very soft central core 31 which may be of fairly 20 high electrical conductivity. If a low conductivity material is used, a separate electrical connection is made to the back of blocking layer 32. This core is coated with a blocking electrode material 32. The blocking electrode layer may be a separate replaceable layer which 25 is either taped on the roller or held by mechanical fasteners or any other device which is capable of releasably holding the layer on the roller; or in the alternative the layer may be integral with the roller itself, being either adhesively bonded, laminated, spray coated or the like on the surface of the roller. It is important that during passage of roller 29 over electrode 11 the two be held together with sufficient force so that the roller material is compressed to provide a flat large area contact 30 between the roller and the electrode 11.

35 In FIGS. 3 and 4, two additional embodiments are illustrated except that the image projector has been left out of these figures to simplify the illustration. In the FIG. 3 embodiment the same NESA glass electrode 11 with a coating of the imaging suspension 14 thereon is employed and is connected to a potential source 17 through a switch 18 as in the previous figures. The other side of potential source 17 is, however, connected to a pair of rollers 36 and 37 and a hold down platen 38 within an elongated endless belt blocking electrode generally designated 39. This endless belt is made up of a base layer 41 with a fairly high electrical conductivity so that the electrical potential applied to the inner rollers and hold down platen will be applied uniformly from this layer through the imaging suspension as the belt passes over electrode 11.

40 As with the central core 31 of roller 29, the substrate 41 of belt 39 may, for example, consist of any suitable

material of relatively high conductivity. Typical conductive materials are conductive rubber, metal foils of steel, aluminum, copper, brass or the like. Blocking electrode layer 42 overlies substrate 41. Rollers 36 and 37 and hold down platen 38 may all be mounted on the same carriage so that movement of the carriage in the direction indicated by the arrow in the drawing will cause electrode 11 to make the desired contact. Hold down platen 38 may also be replaced with a plurality of rollers if desired so as to reduce friction while still pressing the belt surface downwardly during its passage over electrode 11. Other modifications of the apparatus which will also produce a "tracking contact" of the endless belt 39 over electrode 11 will occur to those skilled in the art. Thus, for example, the two rollers and hold down platen may all be replaced with a reinforced block of material having a low coefficient of friction and having the shape as defined by the inside of the belt as seen in FIG. 3, and this block with the belt on its outer surface may simply be slid across electrode 11 so that the same type of tracking is caused to occur. Rotation of the belt in this instance would be caused by the frictional contact of the outer surface of the belt with electrode 11 and the low degree of frictional drag between the belt and the block which would tend to restrict its rotation around the block. In another modification the rollers may be provided with teeth running parallel to their axes adapted to engage ridges cut into the inner surface of the belt so as to provide a positive drive for the belt itself as it tracks over the electrode.

Referring now to FIG. 4, there is seen a third embodiment in which the blocking electrode is supplied in the form of an elongated web 44 provided from a supply roll 46 with a take-up roll 47. This web is entrained over a number of small conductive rollers 48, each of which is connected to potential source 17 so as to provide a good source of electrical potential behind the web as it passes over electrode 11. Rollers 48 along with supply and take-up reels 46 and 47, respectively, are all journaled for rotation on a mounting plate 49. A similar mounting plate may also be provided at the near end of these reels and rollers, as seen in FIG. 4, so that they will be journaled at both ends so as to make up a rigid carriage frame for the whole blocking electrode assembly. In operation, this assembly is moved so as to track the blocking electrode 44 over electrode 11 by following path 51 shown in the figure in dotted line. In this way, the blocking electrode web 44 will track over electrode 11, be lifted up and return back to its original position so that a new section of blocking electrode material will be provided for each pass of this electrode over electrode 11.

The above apparatus and processes are more thoroughly described in U.S. Pat. No. 3,551,320. Examples of other photoelectrophoretic apparatus may be found in U.S. Pat. Nos. 3,565,614 and 3,609,028.

The blocking electrode material which is the subject matter of the present invention is shown in an imaging apparatus environment at 26 in FIG. 1; 32 in FIG. 2; 42 in FIG. 3; and 44 in FIG. 4.

As indicated above, the blocking electrode material of this invention is prepared from a composition comprising a polymeric material having dispersed therein a finely divided ferroelectric material. The term "polymeric" is intended to encompass elastomeric polymers such as natural or synthetic rubber, thermoplastic resins and blends thereof, said polymeric material having

a volume resistivity of at least about  $10^7$  ohm-cm at 23°C. The particular polymer to be used will depend primarily on the demands to be made upon the blocking electrode during the imaging process and the type of apparatus in which the blocking electrode is employed. Where the blocking electrode material is to be used once and then discarded, as could be the case in the scheme of FIG. 4, virtually any polymeric material which can be formed into a sheet or web and which exhibits structural integrity under operating conditions may be used. Exemplary of such materials would be polyolefins such as polyethylene or polypropylene, chlorinated and chlorosulfonated polyolefins, polyacrylates, polyvinyl halides, vinylaromatic polymers such as polystyrene, diene polymers such as natural rubber, polybutadiene, polychloroprene, butyl rubber and ethylene/propylene/diene terpolymers, polyurethanes, polyesters, polyethers and the like. Copolymers of monomers from which the above polymers are derived may also be employed. Where diene or rubbery polymers are used, they should be in the cured state. Best results in terms of image quality are achieved using polymers which, when cast into a sheet or web, exhibit good compliance and flexibility. These characteristics are inherent in elastomeric polymers and can be imparted into more brittle polymers by the use of plasticizers or by blending brittle polymers with elastomeric polymers as is known in the art. Where the blocking electrode material is to be used in a continuous recycling operation as would be the case in the scheme of FIGS. 1, 2 and possibly 3, polymers meeting more stringent requirements in terms of their mechanical and chemical properties should be employed. Good solvent resistance and resistance to abrasion and oxidation are important because of continuous exposure to air and solvents contained in the photoelectrophoretic ink. In addition, the polymer used in forming the blocking layer of the roller electrode as in the scheme of FIG. 1 should be quite compliant so as to assume as nearly as possible the shape of the surface of the injecting electrode as it rolls across the surface of the electrode. Exemplary polymers particularly meeting the above criteria in varying degrees are cured elastomers comprising polyepihalohydrin, copolymers of epihalohydrin with ethylene oxide, polysulfide rubber, silicone rubber, diolefin/acrylonitrile copolymers, polyacrylic rubber, polychloroprene rubber, butyl rubber, chlorosulphonated polyethylene, olefin rubber, fluorinated rubber and like materials and blends thereof.

A second component of the blocking layer of this invention comprises a finely divided ferroelectric material uniformly dispersed in the polymeric matrix. This material functions primarily to increase the dielectric constant of the polymeric layer, thereby enhancing the ability of the polymer to support the high electric field and high flux density generated during the imaging process. It has been found in actual practice that suitable results in the electrophoretic imaging process are obtained when the blocking layer exhibits a dielectric constant of at least about eight. Optimum results are achieved when the dielectric constant of the blocking layer is at least about 15, preferably from about 30 to about 90 or more. This is accomplished according to the present invention by incorporating an amount of finely divided ferroelectric material into the polymeric matrix sufficient to raise the dielectric constant of the polymer composition to a level of about eight or more.

The term ferroelectric material as used herein is intended to refer to those materials having a dielectric constant in excess of 15 ( $10^6$  Hertz) and preferably within the range of from about 100 to 12,000. Exemplary of preferred material are metal titanates and stannates, specifically the alkaline earth metal titanates and stannates.

The amount of ferroelectric material blended with the polymeric material will vary as a factor of the dielectric constant of the particular polymer employed and the dielectric constant of the ferroelectric. Most polymers have a dielectric constant within the range of about 2 to about 7. More of the ferroelectric is required where the polymer has a low initial dielectric constant. In general, from about 20 to about 90 percent by weight ferroelectric based on polymeric material has been found sufficient to increase the dielectric constant of the polymer composition to within the acceptable range. In most cases, a loading of about 50 to 85 percent by weight of the ferroelectric is required in order to impart an optimum dielectric constant of about 30 to 90 into the polymer composition.

The polymeric material and the ferroelectric material may be mixed by any convenient method. The ferroelectric is preferably used in finely divided form, i.e., an average particle size within the range of about 0.1 to 10 microns. Blends may be formed by adding the powdered ferroelectric to a hot melt of the polymeric material in a mill mixer such as a Brabender Plastograph. Mixing may also be carried out using a Banbury mixer which is commonly used in rubber compounding, or by mixing the powder with a polymer latex prior to coagulation and recovery of the latex. Where the polymeric material comprises an elastomer which is to be cured or vulcanized, the appropriate curing agents and rubber processing aids as are known in the art may also be added at this time.

Although blocking electrodes having a blocking layer prepared from the mixture of polymeric material and ferroelectric perform quite well in the electrophoretic process, certain problems may arise where the blocking electrode is intended for use in a continuous process involving cyclic reexposure of the same surface to the high imaging field, as would be the case where the electrode is in the form of a roller as in FIGS. 1 and 2. Residual charge present on the surface of the electrode from a previous cycle must be substantially dissipated before a second cycle commences or the residual charge will interfere with subsequent imaging. In other words, the blocking layer should have a relatively short time constant or relaxation time which should be less than the cycling time but greater than the imaging time. For the purposes of this invention, it has been found that the volume resistivity ( $23^\circ\text{C}$ ) of the blocking layer should be less than about  $10^{13}$  ohm-cm, preferably within the range of about  $10^8$  to  $10^{12}$  ohm-cm, in order for the blocking layer to sufficiently self-discharge residual charges via internal conduction between the use cycles. Thus, where the volume resistivity of the blocking layer comprising the mixture of polymeric material and ferroelectric material is in excess of  $10^{13}$  ohm-cm and the blocking layer is intended for cyclic reuse, the volume resistivity may be lowered to within acceptable limits by intimately mixing with the blocking layer composition minor amounts of an additive which is more conductive than the polymeric material. Exemplary materials suitable for this purpose include conductive fillers

such as graphite and conductive carbon black, Lewis acids, polyelectrolytic resins such as QX2611.12 which is a polyquaternary ammonium salt complex available from Dow Chemical Co., plasticizers such as triphenyl or tricresyl phosphate or N-ethyl p-toluenesulphonamide, polymer curing agents, and impurities such as organic dyes and halogen molecules. In general, the conductive additive should have a volume resistivity of less than  $10^6$  ohm-cm ( $23^\circ\text{C}$ ) and preferably less than  $10^3$  ohm-cm, and may be used at a level of from about 0.1 to about 25 percent by weight, based on the weight of polymeric material.

The above compositions may be fabricated into a blocking layer for use in conjunction with a blocking electrode by any one of a number of techniques. The polymeric blocking layer may be applied to the appropriate conductive substrate directly by dip or roller coating. Alternatively, sheets or films of the polymeric materials may be prepared by casting films or by compression molding, and these applied to the substrate by adhesive lamination or by heat shrinking where the polymeric material is one susceptible to heat shrinkage. Where the polymeric material is an elastomer which is to be cured prior to use as a blocking layer, the elastomer containing the appropriate curing agents may be cured in situ after application to the conductive substrate, or films and sheets of the elastomer may be formed, cured and subsequently applied to the conductive substrate. In another embodiment, the polymeric blocking layer may be fabricated into a web or sheet which is adapted to be fed into ultimate contact with a conductive substrate during the imaging process. These webs or sheets may be prepared by continuous film casting processes, extrusion, solvent deposition and like techniques known to those skilled in the art. Webs and sheets may also be prepared by forming a thin continuous coating of the polymeric composition on a relatively inert substrate such as paper or by saturating a loose matrix such as paper prior to calendering.

The thickness of the blocking layer may vary within wide limits, but should be substantially uniform for best results. The minimum thickness is determined by practical considerations such as the particle size of the various additives present in the blocking layer composition and the ability to cast uniform films without the formation of irregularities or pinholes. The upper limit of film thickness is limiting in the sense that the total potential established between the injection and blocking electrodes must be maintained by increasing the voltage as a function of the thickness of the blocking layer. For the purposes of this invention the substantially uniform thickness of the blocking layer should be at least 1 mil, preferably within the range of about 5 mils to about one-fourth inch, and more preferably within the range of about 10 to 50 mils.

The conductive support underlying the blocking layer may comprise any suitably conductive material such as metal or conductive rubber, or a sleeve of conductive rubber overlying a metal core. The conductive support in turn is connected to a source of potential. Where the blocking electrode is in the form of a roller as in FIGS. 1 and 2, the use of conductive rubber imparts added compliance to the roller electrode.

The following examples are illustrative of compositions suitable for use as a blocking layer and methods for preparing them.

## Example I

The following materials were mixed and compounded on a rubber mill:

| Parts by Weight                                |                    |
|------------------------------------------------|--------------------|
| Butadiene/acrylonitrile copolymer (Hycar 1043) | 100.0              |
| Stearic acid                                   | 1.0                |
| Zinc oxide                                     | 5.0                |
| Barium titanate powder*                        | 40.0               |
| Tetramethyl thiuram disulfide                  | 3.5                |
| * Capacitor grade barium titanate              |                    |
| Specific gravity                               | 5.85               |
| Bulk density                                   | 124 lb/cu ft       |
| Melting point                                  | 3010°F             |
| Fineness                                       | 0.3 to 5.0 microns |
| Dielectric constant<br>(10 <sup>6</sup> Hertz) | 1200-1600          |

A cured film comprising the above composition having a thickness of about 25 mils was prepared by curing the composition in a mold in a hydraulic press at 350°F for 15 minutes. The cured film exhibited a dielectric constant of about 15 and a volume resistivity in the order of 10<sup>10</sup> ohm-cm.

The film was bonded to a conductive roller substrate like that shown at 24 in FIG. 1 having a diameter of about 4 inches and a length of about 12 inches. Excellent images were produced using this assembly as the blocking electrode.

## EXAMPLE II

The following materials were mixed and compounded on a rubber mill:

| Parts by Weight                  |        |
|----------------------------------|--------|
| Polyepichlorohydrin (Hydrin 100) | 100.0  |
| Magnesium stearate               | 1.0    |
| Lead phosphate (dibasic)         | 7.5    |
| Hexamethylidamine carbamate      | 0.8    |
| Phenol salicylate powder         | 0.5    |
| Barium titanate powder           | 300.00 |

A cured film having a thickness of about 20 mils was prepared by curing the composition in a hydraulic press at 280°F for one hour. The film exhibited a dielectric constant of about 60 and a resistivity of about 10<sup>10</sup> ohm-cm.

A blocking electrode similar to that shown in FIG. 3 is constructed by laminating a length of film prepared as above 42 to a  $\frac{1}{8}$  inch thick belt comprising conductive rubber 41 containing a high loading of carbon black. As in Example I, the blocking electrode produced excellent images when used in the electrophoretic imaging process.

## EXAMPLE III

A film having a thickness of about 20 mils and exhibiting excellent imaging characteristics when used as a blocking layer in a blocking electrode was prepared by compounding and curing the following composition as in Example II:

| Parts by Weight                                 |       |
|-------------------------------------------------|-------|
| Chlorosulphonated polyethylene (Dupont Hypalon) | 100.0 |
| Litharge                                        | 25.0  |
| Dipentamethylene thiuramtetrasulfide            | 1.0   |
| N,N-m-phenylene dimaleimide                     | 1.0   |
| Barium titanate powder                          | 300.0 |

The film exhibited a dielectric constant of about 70 and a resistivity of about 10<sup>9</sup> ohm-cm. The N,N-m-phenylene dimaleimide functions in this formula both as a curing aid and a conductive material. Without this material, a resistivity in the order of 10<sup>13</sup> ohm-cm would be expected.

## EXAMPLE IV

A film having a thickness of about 20 mils was prepared by compounding and curing the following composition as in Example II:

| Parts by Weight                   |       |
|-----------------------------------|-------|
| 15 Chlorosulphonated polyethylene | 40.0  |
| Polyepichlorohydrin               | 60.0  |
| Magnesium oxide                   | 4.0   |
| Zinc oxide                        | 1.0   |
| Barium/cadmium soap (Ferro 1827)  | 2.0   |
| Barium titanate powder            | 280.0 |
| 2-mercaptopimidazoline            | 1.2   |
| N,N-m-phenylene dimaleimide       | 0.6   |

The film exhibited a dielectric constant of about 65 and a resistivity of about 10<sup>10</sup> ohm-cm.

## EXAMPLE V

In this example, carbon black is used to lower the volume resistivity of the composition to less than 10<sup>12</sup> ohm-cm. A film having a thickness of about 25 mils was prepared by compounding and curing the following composition as in Example II:

| Parts by Weight                                |       |
|------------------------------------------------|-------|
| Chlorosulphonated polyethylene                 | 100.0 |
| Magnesium oxide                                | 4.0   |
| Barium titanate powder                         | 280.0 |
| Dipentamethylene thiuramtetrasulfide           | 2.5   |
| Mercaptobenzothiazyl disulfide                 | 0.5   |
| Carbon black                                   | 20.0  |
| 40 Epoxy resin (Epon 828 — Shell Chemical Co.) | 4.0   |

This film produced excellent imaging when used in conjunction with a roller electrode as in Example I.

## EXAMPLE VI

The following ingredients were dispersed in cellosolve acetate solvent at about 35 percent by weight solids:

| Parts by Weight                                |               |
|------------------------------------------------|---------------|
| Polyurethane resin*                            | 25.0          |
| Strontium titanate**                           | 75.0          |
| * Chemglaze — Hughson Chemical Company         |               |
| ** National Lead Company                       |               |
| Specific gravity                               | 4.81          |
| Bulk density                                   | 84            |
| Melting point                                  | 7340°F        |
| Fineness                                       | 0.563 microns |
| Dielectric constant<br>(10 <sup>6</sup> Hertz) | 225-250       |

60 The dispersion was sprayed evenly on the surface of a stainless steel roller electrode similar to that shown in FIG. 1 in amounts sufficient to form a coating having a dried film thickness of about 2 mils. The film exhibited a dielectric constant of about 9 and a resistivity of about 10<sup>14</sup> ohm-cm. The resultant blocking electrode produced a good image when subjected to single cycle imaging in the electrophoretic imaging process.

Suitable blocking layers for use in the electrophoretic imaging process may also be prepared from blends comprising a mixture of thermoplastic material such as polymethylmethacrylate, polystyrene, polyvinyl fluoride, polyvinylidene fluoride, polyethylene, polypropylene and the like and from about 20 to 90 percent by weight of finely divided ferroelectric material such as barium titanate or strontium titanate. These compositions may be applied in thicknesses ranging from about 1 mil to  $\frac{1}{4}$  inch by spraying, dipping or roller coating to any suitable substrate such as the conductive roller 24 of FIG. 1, the conductive roller 31 of FIG. 2, or conductive belt 41 of FIG. 3. Alternatively, the composition may be formed into a web of the same thickness as indicated at 44 of FIG. 4.

What we claim is:

1. A blocking electrode for use in a photoelectrophoretic imaging process comprising:
  - a conductive support having means for coupling to an electrical energy source;
  - b. a polymeric layer in contact with said conductive support;
 said polymeric layer comprising a polymeric material having from about 20 to about 90 percent by weight of a finely divided ferroelectric material dispersed therein, said ferroelectric material having a dielectric constant of at least about 15.
2. The blocking electrode of claim 1 wherein said polymeric layer is adapted for interposition between the conductive support and a second electrode.
3. The blocking electrode of claim 2 wherein said ferroelectric material is selected from the group consisting of alkaline earth metal titanates and alkaline earth metal stannates.
4. The blocking electrode of claim 3 wherein said polymeric layer is in the form of a sheet adapted for feeding between said conductive support and said second electrode.
5. The blocking electrode of claim 3 wherein said conductive support comprises a cylinder or continuous belt having said polymeric layer wrapped about the external periphery thereof.
6. The blocking electrode of claim 5 wherein said polymeric material comprises a cured elastomer.
7. The blocking electrode of claim 6 wherein said polymeric layer has a dielectric constant of at least about 15 and a volume resistivity within the range of about  $10^8$  to  $10^{12}$  ohm-cm.

8. The blocking electrode of claim 7 wherein the polymeric layer further contains from about 0.1 to about 25 percent by weight of a conductive material having a volume resistivity of less than about  $10^6$  ohm-cm.

9. The blocking electrode of claim 8 wherein said conductive material comprises carbon black.

10. The blocking electrode of claim 6 wherein the cured elastomer is selected from the group consisting of butadiene/acrylonitrile rubber, chlorosulfonated polyethylene, epichlorohydrin polymers and mixtures thereof.

11. A blocking electrode for use in a photoelectrophoretic imaging process comprising:

- a conductive support having means for coupling to an electrical energy source;
- a polymeric layer in contact with said conductive support and interposed between said conductive support and a second electrode;
- said polymeric layer comprising a uniform mixture of a polymeric material having a volume resistivity of greater than about  $10^7$  ohm-cm and a finely divided ferroelectric material selected from the group consisting of barium titanate, strontium titanate and mixtures thereof,
- said ferroelectric material present in an amount sufficient such that the polymeric layer has a dielectric constant of at least about eight.
12. The blocking electrode of claim 11 wherein said polymeric layer has a dielectric constant of at least about 15 and is of substantially uniform thickness within the range of from about 1 mil to  $\frac{1}{4}$  inch.
13. The blocking electrode of claim 12 wherein said conductive support comprises a cylinder or continuous belt having said polymeric layer wrapped around the external periphery thereof, the thickness of said polymeric layer being at least about 5 mils.
14. The blocking layer of claim 13 wherein said polymeric material is a cured elastomer selected from the group consisting of butadiene/acrylonitrile rubber, chlorosulfonated polyethylene, epichlorohydrin polymers and mixtures thereof.
15. The blocking electrode of claim 11 wherein the ferroelectric material is barium titanate having a particle size within the range of about 0.1 to 10 microns, said barium titanate present at a level of from about 20 to 90 percent by weight of the polymeric material.

\* \* \* \* \*